

## UNITED STATES PATENT OFFICE

2,576,896

COMPOSITIONS OF MATTER FOR PRODUC-  
ING A SOFTENING EFFECT ON TEXTILESOtto Albrecht, Neuewelt, Switzerland, assignor to  
Ciba Limited, Basel, Switzerland, a Swiss firmNo Drawing. Application June 19, 1947, Serial  
No. 755,709. In Switzerland June 28, 1946

4 Claims. (Cl. 252—8.75)

1

According to this invention, fibrous materials are softened in an advantageous manner by treating the material with an aqueous dispersion of a partial ester of a higher fatty acid and a glycol, which dispersion contains as a dispersing agent a water-soluble salt of a condensation product of an N-methylolamide of a higher fatty acid with a mercapto-carboxylic acid and, if desired, a lime-resistant sulfonation product of a benzimidazole having attached to the  $\mu$  carbon atom a side-chain of at least 12 carbon atoms.

As partial esters of fatty acids of high molecular weight which are used in the invention in dispersed form, there may be mentioned esters of ethylene glycol, diethylene glycol, triethylene glycol or even higher polyglycols with fatty acids of high molecular weight, especially fatty acids containing at least 12 carbon atoms. Polyglycols as mentioned above correspond to the formula



wherein  $x$  is at least one.

As condensation products of N-methylolamides of higher fatty acids with mercapto-carboxylic acids, there may be used, for example, condensation products of the formula



wherein  $x$  is an amino group acylated with a fatty acid with at least 16 carbon atoms and  $R$  is alkylene. Examples of condensation products of this kind are, for instance, the condensation products obtainable from thioglycolic acid and palmitic acid N-methylolamide, stearic acid, N-methylolamide or oleic acid-N-methylolamide, which contain the atomic grouping



in which



is the acyl residue of the fatty acid used. Examples of condensation products with the aforementioned atomic grouping are compounds of the formulae



and

2



wherein

15



is the acyl radical of the fatty acid employed in the condensation. Products of these constitutions are described in U. S. Patent No. 2,337,220.

These examples demonstrate that an acylated amino group corresponds to the formula



wherein

30



is an acyl radical of a carboxylic acid and  $R_1$  is hydrogen or a hydrocarbon radical, for instance, an alkyl radical which may be substituted;  $R_1$  may be, for instance, methyl, ethyl or a methyl radical substituted by an acylated amino group. As an example of this kind of substituted methyl radicals the following may be cited:



40

wherein  $-\text{CO}-\text{R}$  has the meaning given above.

As lime-resistant sulfonation products of a benzimidazole having attached to the  $\mu$  carbon atom a side-chain of at least 12 carbon atoms, the dispersions used in the invention may contain, for example, the following products: Sulfonic acids of benzimidazoles having attached to the  $\mu$ -carbon atom a side chain of at least 12 carbon atoms, which benzimidazoles may, if desired, be aralkylated, for example, the sodium salt of N-benzyl- $\mu$ -heptadecyl-benzimidazole di-

45

sulfonic acid.

In order to prepare the dispersions to be used in the invention, the partial esters of higher fatty acids and a glycol may be introduced, advantageously in the molten state in the case of compounds which are solid at room temperature, into concentrated solutions or pastes of the above mentioned dispersing agents while rapidly stir-

50

3

ring, advantageously at a temperature above the melting point of the substance to be dispersed.

The dispersions of the present invention may be described as compositions of matter producing a softening effect on textiles which compositions of matter comprise an aqueous dispersion of a partial ester of a higher fatty acid and a glycol, said dispersion containing a water-soluble salt of a condensation product of an N-methylolamide of a higher fatty acid with a mercapto-carboxylic acid.

The softening process of the invention may be carried out by impregnating the material at room temperature or a moderately raised temperature with an aqueous liquor containing a small quantity of a dispersion of the kind described above, for example, 1 to 5 grams per liter, and then squeezing or centrifuging the material and drying it.

Among the fibrous materials which can be softened by the process of the invention there may be mentioned: Animal fibers such as wool or silk; cellulosic materials such as cotton, linen, cellulose, paper, and also regenerated cellulose including staple fibers of regenerated cellulose; cellulose acetate artificial silk; synthetic materials produced, for example, by polymerisation or condensation, for example, polyamide fibers; and also leather.

The following examples illustrate the invention, the parts being by weight unless otherwise stated, and the relationship of parts by weight to parts by volume being the same as that of the kilogram to the liter:

#### Example 1

Chlorinated wool is softened in the following manner:

A bath is prepared which contains, per liter, 1 gram of a mixture of 25 parts of diethylene glycol monostearate, 14 parts of the sodium salt of a carboxylic acid obtainable by the condensation of stearic acid-N-methylolamide with thioglycollic acid and also 11 parts of the disodium salt of N-benzyl- $\mu$ -heptadecyl-benzimidazole disulfonic acid. The wool is worked in the bath at a liquor ratio of 1:10 for  $\frac{1}{4}$  hour at room temperature and centrifuged and dried. The wool so obtained is distinctly softer than the untreated material.

The dispersion used above is prepared in the following manner:

168 parts of the sodium salt of the carboxylic acid obtainable by condensing stearic acid-N-methylolamide with thioglycollic acid, and 72 parts of the disodium salt of N-benzyl- $\mu$ -heptadecyl-benzimidazole disulfonic acid are added in portions while stirring to 100 parts by volume of water at 95° C. Then a further 60 parts of the disodium salt of N-benzyl- $\mu$ -heptadecyl-benzimidazole disulfonic acid are introduced while stirring, advantageously with the introduction of steam heated to 100° C. In the course of about 30 minutes 300 parts of diethylene-glycol monostearate heated at 90° C. will have been stirred into the homogeneous paste so obtained. The stirring is continued for a short time, then the temperature is allowed to drop to 60° C., and its weight is made up to 1200 parts, and the whole is then allowed to cool while stirring. In order to prepare the treatment bath the concentrated dispersion is boiled with 10 times its weight of water and then further diluted.

The condensation product of stearic acid-N-

methylolamide and thioglycollic acid as used above corresponds to the formula



and is obtained by condensing one molecular proportion of the methyloamide of commercial stearic acid with  $\frac{1}{2}$  molecular proportion of thioglycollic acid.

A similar effect can be obtained by using, instead of diethylene glycol monostearate, the corresponding oleic acid ester and in other respects working exactly in the manner described above.

#### Example 2

Wool is softened in the following manner: A bath is prepared which contains, per liter, 1.25 grams of a stearic acid polyglycol ester obtained by condensing 1 molecular proportion of commercial stearic acid with 3.8 molecular proportions of ethylene oxide, and also 0.875 gram of the sodium salt of the carboxylic acid obtainable by the condensation of stearic acid-N-methyloamide with thioglycollic acid and 0.375 gram of the disodium salt of N-benzyl- $\mu$ -heptadecyl-benzimidazole disulfonic acid. The wool is worked in the bath at a liquor ratio of 1:10 for  $\frac{1}{4}$  hour at room temperature and centrifuged and dried. The wool so obtained is distinctly softer than the untreated material.

The stearic acid polyglycol ester used above can be obtained by forcing 247.5 parts of ethylene oxide under a pressure of 6 to 10 atmospheres at 150-155° C. into 400 parts of commercial stearic acid and 15.1 parts of finely ground sodium acetate.

The dispersion used above may be prepared as follows: 525 parts of the sodium salt of the carboxylic acid obtainable by the condensation of stearic acid N-methyloamide with thioglycollic acid and 225 parts of the disodium salt of N-benzyl- $\mu$ -heptadecyl-benzimidazole disulfonic acid are heated at the boil with 375 parts of water, while stirring. In this manner a homogeneous paste is obtained. 750 parts of the above described stearic acid polyglycol ester heated to 90° C. are then introduced in small portions in the course of 30 minutes while rapidly stirring. The resulting homogeneous paste is stirred cold and made up to a weight of 3000 parts by the addition of water.

A similar effect can be obtained by using, instead of the above mentioned stearic acid polyglycol ester, the oleic acid polyglycol ester obtainable from 1 molecular proportion of oleic acid and 6 molecular proportions of ethylene oxide.

What I claim is:

1. Composition of matter producing a softening effect on textiles and consisting of an aqueous dispersion of a partial ester of a fatty acid with at least 12 carbon atoms and a member selected from the group consisting of a glycol and a glycol ether of the formula



wherein  $x$  is at least one, said dispersion containing a water-soluble salt of a carboxylic acid of the formula



wherein  $\text{R}'-\text{CO}-$  is the acyl radical of a fatty acid with at least 16 carbon atoms, said dispersion

containing also a water-soluble salt of a sulfonated benzimidazole in which the  $\mu$  carbon atom of the imidazole ring is bound to an alkyl radical of at least 12 carbon atoms, the relative proportions of the ingredients being about 50 parts by weight of the ester to 28-35 parts by weight of the water-soluble salt of the carboxylic acid and 15-22 parts by weight of the water-soluble salt of the sulfonated benzimidazole.

2. Composition of matter producing a softening effect on textiles and consisting of an aqueous dispersion of a partial ester of a fatty acid with at least 12 carbon atoms and a glycol, said dispersion containing a water-soluble salt of a carboxylic acid of the formula



wherein  $R'$ —CO— is the acyl radical of a fatty acid with at least 16 carbon atoms, said dispersion containing also a water-soluble salt of a sulfonated benzimidazole in which the  $\mu$ -carbon atom of the imidazole ring is bound to an alkyl radical of at least 12 carbon atoms, the relative proportions of the ingredients being about 50 parts by weight of the ester to 28-35 parts by weight of the water-soluble salt of the carboxylic acid and 15-22 parts by weight of the water-soluble salt of the sulfonated benzimidazole.

3. Composition of matter producing a softening effect on textiles and consisting of an aqueous dispersion of a partial ester of a fatty acid with at least 12 carbon atoms and a glycol ether of the formula



wherein  $x$  is at least one, said dispersion containing a water-soluble salt of a carboxylic acid of the formula



wherein  $R'$ —CO— is the acyl radical of a fatty acid with at least 16 carbon atoms, said dispersion containing also a water-soluble salt of a sulfonated benzimidazole in which the  $\mu$ -carbon atom of the imidazole ring is bound to an alkyl radical of at least 12 carbon atoms, the relative proportions of the ingredients being about 50 parts by weight of the ester to 28-35 parts by weight of the water-soluble salt of the carboxylic acid and 15-22 parts by weight of the water-soluble salt of the sulfonated benzimidazole.

4. Composition of matter producing a softening

effect on textiles and consisting of an aqueous dispersion of an ester of the formula



5. wherein R—CO— is the acyl radical of commercial stearic acid, said dispersion containing a water-soluble salt of the carboxylic acid of the formula



wherein  $R'$ —CO— is the acyl radical of commercial stearic acid, this carboxylic acid being obtained by condensing 1 molecular proportion of the methylol amide of commercial stearic acid with  $\frac{1}{2}$  molecular proportion of thioglycollic acid, said dispersion containing also a water-soluble salt of a disulfonic acid of the benzimidazole of the formula



wherein R is the alkyl radical contained in commercial stearic acid of the formula



25 the relative proportions of the ingredients being about 50 parts by weight of the ester to 28-35 parts by weight of the water-soluble salt of the carboxylic acid and 15-22 parts by weight of the water-soluble salt of the sulfonated benzimidazole.

OTTO ALBRECHT.

#### REFERENCES CITED

The following references are of record in the file of this patent:

#### UNITED STATES PATENTS

| Number       | Name      | Date          |
|--------------|-----------|---------------|
| 1,985,687    | Nuesslein | Dec. 25, 1934 |
| 2,036,525    | Granacher | Apr. 7, 1936  |
| 50 2,043,164 | Granacher | June 2, 1936  |
| 2,245,412    | Pilgrim   | June 10, 1941 |
| 2,337,220    | Albrecht  | Dec. 21, 1943 |
| 2,345,632    | Robinson  | Apr. 4, 1944  |

#### OTHER REFERENCES

Chem. Glycols, pub. by Glyco Product Co., copyright 1948, p. 12.